

## UNITED STATES PATENT OFFICE

2,580,587

MINERAL OIL COMPOSITION CONTAIN-  
ING A POLYMERICALKYL METAPHOS-  
PHIMATE

Ferdinand P. Otto, Woodbury, and Robert W. Barrett, Sewell, N. J., assignors to Socony-Vacuum Oil Company, Incorporated, a corporation of New York

No Drawing. Application November 14, 1949,  
Serial No. 127,268

4 Claims. (Cl. 252—49.9)

1

This invention relates generally to improved lubricating oil compositions and more particularly to lubricating oil compositions having advantageously low pour points.

As is well known, mineral lubricating oils, particularly those derived from paraffin base crudes, tend to congeal and become non-flowing at temperatures slightly below normal atmospheric temperatures. This is due to the crystallization of the wax content of the oil and, of course, is undesirable, particularly if the oil is to be utilized in automotive engines in temperate climates where temperatures normally encountered in winter cause the oil to congeal in the crankcase when the engine is idle. As a result, when the engine is started cold, it is subjected to conditions of increased wear and breakdown, since the parts do not receive proper lubrication. It is known, however, that this condition may be counteracted by adding to the oil small amounts of certain chemical compounds which inhibit the crystallization of the wax content therein and thus effect a considerable lowering of the temperature at which the oil will cease to flow. Such compounds are known as pour point depressants. The present invention is concerned with oil compositions containing additive compounds of this type.

We have found that when a minor proportion of a polymer product obtained by first condensing a phosphonitrilic halide with an alcohol selected from the class consisting of n-tetradecanol and a mixture of primary, normal, saturated, aliphatic alcohols having an average of about 14 carbon atoms per molecule and then subjecting the condensation product so produced to polymerizing conditions, is added to a mineral lubricating oil, the pour point of the oil is lowered to a considerable extent.

It is, therefore, an object of this invention to provide mineral lubricating oil compositions of lowered pour point, said compositions containing small amounts of the aforesaid type of polymer product. Other objects will appear from the following detailed description of the invention.

The condensation products which are polymerized to produce the oil addition agents contemplated herein are alkyl metaphosphimates. It has been known heretofore that these materials could be polymerized. Thus, Patent No. 2,214,769 describes the polymerization of similar compounds obtained by the condensation of phosphonitrilic halides with organic compounds such as methyl, ethyl, propyl, butyl and amyl alcohols. No mention is made in that patent, however, of the particular polymerization products herein contemplated, viz. those obtained

2

by polymerizing an alkyl metaphosphimate derived from a primary, normal, saturated alcohol having 14 carbon atoms or from a mixture of primary, normal, saturated alcohols having an average of approximately 14 carbon atoms per molecule; nor does the patent suggest the utility of such polymers as pour point depressants in mineral oils.

Another patent, No. 2,109,491, describes lubricating oil compositions containing condensation products of metaphosphimates obtained from certain other aliphatic alcohols, including lauryl, dodecyl and oleyl alcohols. However, no mention is made of metaphosphimates produced from the alcohols useful in this invention, viz. n-tetradecanol, or a mixture of primary, normal, saturated alcohols having an average of 14 carbon atoms per molecule. Furthermore, there is no disclosure to the effect that when the latter compounds are subjected to polymerizing conditions as hereinafter defined, reaction products are obtained which are effective as pour point depressants in mineral lubricating oils.

As indicated hereinbefore, in accordance with this invention, a phosphonitrilic halide, particularly a phosphonitrilic chloride, comprised substantially of  $(\text{PNCl}_2)_3$  and  $(\text{PNCl}_2)_4$ , is first condensed with either n-tetradecyl alcohol, or of a mixture of primary, normal, saturated alcohols having an average of about 14 carbon atoms per molecule at a relatively low temperature, i. e. not over about 150° C., to form a condensation product. The condensation reaction is more efficient if the alcohol is first converted to a metal alcoholate of a metal such as sodium or potassium. The condensation reaction, when employing  $(\text{PNCl}_2)_3$  and sodium tetradecanolate, for example, is represented by the following equation:



At the aforesaid condensation temperature, substantially no polymerization of the phosphonitrilic chloride will occur. The condensation product is then polymerized by heating at higher temperatures, for example, from about 200° C. up to about 400° C., or by further heating at the lower temperatures in the presence of a suitable polymerization catalyst, such as  $\text{AlCl}_3$ ,  $\text{ZnCl}_2$ ,  $\text{BF}_3$  and the like. We have found it convenient to carry out the reaction in the presence of about 5 per cent by weight of  $\text{AlCl}_3$ , using xylene as a solvent and maintaining the temperature at the reflux temperature of the solvent.

Although the phosphonitrilic chlorides are par-

3  
ticularly contemplated herein, the phosphonitrilic dibromides and iodides may also be used.

As indicated above, the alcohols capable of providing polymeric products of the type contemplated herein are tetradecanol or a mixture of primary, normal, saturated, aliphatic alcohols having an average of approximately 14 carbon atoms per molecule. Such a mixture of alcohols, for example, is that marketed by E. I. du Pont de Nemours & Co. under the trade name "Lorol-B." This is a mixture of alcohols, containing primary, normal, saturated, aliphatic alcohols in approximately the following proportions:

| Per cent              |
|-----------------------|
| C <sub>10</sub> = 2.5 |
| C <sub>12</sub> =55.0 |
| C <sub>14</sub> =20.5 |
| C <sub>16</sub> = 9.0 |
| C <sub>18</sub> =13.0 |
| Ave. No. C Atoms=13.5 |

The following examples and results of tests will serve to illustrate more fully the principles of our invention.

#### PREPARATION OF PHOSPHONITRILIC CHLORIDE

Reaction mixture:

|                               |       |      |
|-------------------------------|-------|------|
| Ammonium chloride             | grams | 130  |
| Phosphorus pentachloride      | do    | 400  |
| Symmetrical tetrachloroethane | cc    | 1000 |

Procedure.—The reactants and solvent were placed in a 3-neck round bottom flask equipped with a reflux condenser, thermometer and mechanically driven stirrer. The resulting mixture was refluxed at 136° C. to 142° C. for a period of 7 hours. After cooling, the mixture was filtered to remove excess ammonium chloride, and the filtrate topped to 55° C. at 11 mm. pressure to remove 850 cc. of tetrachloroethane. On cooling the residue in an ice-salt bath, the product consisting of essentially (PNCl<sub>2</sub>)<sub>3</sub> and (PNCl<sub>2</sub>)<sub>4</sub> crystallized from the mixture and was filtered therefrom. After washing with cold tetrachloroethane, the material contained on the filter weighed 87 grams and by analysis contained 12.1 per cent nitrogen (theor.=12.0%).

#### EXAMPLE I

*Reaction product of phosphonitrilic chloride with Sodium "Lorol-B" alcoholate*

Reaction mixture:

|                          |       |      |
|--------------------------|-------|------|
| Metallic sodium          | grams | 5.0  |
| Butanol                  | cc    | 100  |
| "Lorol-B"                | grams | 47.0 |
| Phosphonitrilic chloride | do    | 11.6 |
| Xylene                   | cc    | 100  |

Procedure.—Metallic sodium was added to the butyl alcohol contained in a round bottom flask equipped with a thermometer, reflux condenser and mechanically driven stirrer. After the sodium had completely reacted to form the sodium butylate, the "Lorol-B" alcohol was added and the n-butyl alcohol permitted to distill from the mixture until the temperature reached 143° C. The sodium salt of the "Lorol-B" alcohol was then mixed with 100 cc. of xylene and the phosphonitrilic chloride consisting essentially of (PNCl<sub>2</sub>)<sub>3</sub> and (PNCl<sub>2</sub>)<sub>4</sub>. After refluxing at 140–145° C. for a period of 6 hours, the mixture was made acidic with dilute HCl and then water washed until neutral. The solvent was then removed from the product by distillation to a temperature of 175° C. at 5 mm. The "Lorol-B"

metaphosphimate so obtained contained 6.58% phosphorus (theor.=6.1%) and 2.97% nitrogen (theor.=3.0%).

#### EXAMPLE I-A

##### *Poly "Lorol-B" Metaphosphimate*

Reaction mixture:

|                             |       |      |
|-----------------------------|-------|------|
| "Lorol-B" metaphosphimate   | grams | 18.0 |
| (Example I)                 |       |      |
| Anhydrous aluminum chloride | do    | 0.9  |

Xylene

Procedure.—The above mixture was placed in a 3-neck round bottom flask equipped with a reflux condenser, thermometer and mechanically driven stirrer. After heating for a period of 9 hours at 125° C. the reaction product was washed with water until the washings were neutral. This was followed by topping to 175° C. at 5 mm. to remove the solvent and obtain the finished product, a semi-viscous yellow oil.

The procedures for preparing the following products were essentially the same as those described in Examples I and I-A.

#### EXAMPLE II

##### *Didecyl Metaphosphimate*

Reaction mixture:

|                          |       |      |
|--------------------------|-------|------|
| Metallic sodium          | grams | 5.0  |
| n-Butyl alcohol          | cc    | 100  |
| 1-decanol                | grams | 60   |
| Xylene                   | cc    | 100  |
| Phosphonitrilic chloride | grams | 11.6 |

#### EXAMPLE II-A

##### *Poly decyl metaphosphimate*

Reaction mixture:

|                             |       |      |
|-----------------------------|-------|------|
| Decyl metaphosphimate       | grams | 16.0 |
| (Example II)                |       |      |
| Anhydrous aluminum chloride | do    | 0.8  |
| Xylene                      | cc    | 50   |

#### EXAMPLE III

##### *Dodecyl metaphosphimate*

Reaction mixture:

|                          |       |      |
|--------------------------|-------|------|
| Metallic sodium          | grams | 5.0  |
| Butanol                  | cc    | 100  |
| 1-dodecanol              | grams | 40   |
| Xylene                   | cc    | 100  |
| Phosphonitrilic chloride | grams | 11.6 |

#### EXAMPLE III-A

##### *Poly dodecyl metaphosphimate*

Reaction mixture:

|                             |       |      |
|-----------------------------|-------|------|
| Dodecyl metaphosphimate     | grams | 16.0 |
| (Example III)               |       |      |
| Anhydrous aluminum chloride | do    | 0.8  |

Xylene

#### EXAMPLE IV

##### *Tetradecyl metaphosphimate*

Reaction mixture:

|                          |       |      |
|--------------------------|-------|------|
| Metallic sodium          | grams | 5.0  |
| Butanol                  | cc    | 100  |
| 1-tetradecanol           | grams | 46.0 |
| Xylene                   | cc    | 150  |
| Phosphonitrilic chloride | grams | 11.6 |

#### EXAMPLE IV-A

##### *Poly tetradecyl metaphosphimate*

Reaction mixture:

|                             |       |      |
|-----------------------------|-------|------|
| Tetradecyl metaphosphimate  | grams | 16.0 |
| (Example IV)                |       |      |
| Anhydrous aluminum chloride | do    | 0.8  |

Xylene

**EXAMPLE V**  
*Hexadecyl metaphosphimate*

## Reaction mixture:

|                          |       |      |    |
|--------------------------|-------|------|----|
| Metallic sodium          | grams | 5.0  | 5  |
| Butanol                  | cc    | 150  |    |
| 1-hexadecanol            | grams | 53   |    |
| Xylene                   | cc    | 100  |    |
| Phosphonitrilic chloride | grams | 11.6 | 10 |

**EXAMPLE V-A**  
*Poly hexadecyl metaphosphimate*

## Reaction mixture:

|                             |       |      |    |
|-----------------------------|-------|------|----|
| Hexadecyl metaphosphimate   | grams | 16.0 | 15 |
| (Example V)                 |       |      |    |
| Anhydrous aluminum chloride | do    | 0.8  |    |

|        |    |    |  |
|--------|----|----|--|
| Xylene | cc | 50 |  |
|--------|----|----|--|

**EXAMPLE VI**  
*Octadecyl metaphosphimate*

## Reaction mixture:

|                          |       |      |    |
|--------------------------|-------|------|----|
| Metallic sodium          | grams | 5.0  | 15 |
| Butanol                  | cc    | 100  |    |
| 1-octadecanol            | grams | 58.0 | 20 |
| Xylene                   | cc    | 100  |    |
| Phosphonitrilic chloride | grams | 11.6 | 25 |

**EXAMPLE VI-A**  
*Poly octadecyl metaphosphimate*

## Reaction mixture:

|                             |       |      |    |
|-----------------------------|-------|------|----|
| Octadecyl metaphosphimate   | grams | 20.0 | 15 |
| (Example VI)                |       |      |    |
| Anhydrous aluminum chloride | do    | 0.9  |    |

|        |    |    |    |
|--------|----|----|----|
| Xylene | cc | 50 | 20 |
|--------|----|----|----|

## POUR POINT DEPRESSION

In order to demonstrate the effectiveness of the particular group of polymer products contemplated by this invention as pour point depressants for mineral lubricating oils, the various products prepared as described in the foregoing examples were blended, in minor proportions, with a typical lubricating oil and the blends subjected to tests to ascertain the pour points thereof. The oil used in all of these blends was a solvent-refined Mid-continent SAE 30 grade stock having an initial pour point of 20° F. and a kinematic viscosity at 210° F. of 11.96. The test results are presented in Tables I and II:

Table I shows the results obtained with blends of a number of monomeric alkyl metaphosphimates produced by merely condensing phosphonitrilic chloride (consisting substantially of  $(\text{PNCl}_2)_3$  and  $(\text{PNCl}_2)_4$ ) with various primary, normal, saturated, aliphatic alcohols containing from 10 to 18 carbon atoms including a product obtained from a mixture of primary, normal, saturated, aliphatic alcohols having an average of about 14 carbon atoms per molecule, i. e. "Lorol-B." It will be seen from the data that none of these provide any significant pour point depressant effect.

Table II shows the results obtained with oil blends of the polymerized products shown in Table I. It will be seen that only the monomeric products prepared from n-tetradecanol and the "Lorol-B" alcohol mixture provide polymerized products which are significantly effective pour point depressants.

The amount of the polymeric alkyl metaphosphimate product to be added to the mineral lubricating oil will vary somewhat with the intended application of the oil composition, but generally will range from about .1 per cent to about 10 per cent. However, significant improvement may be obtained with lesser amounts. It is also contemplated that the product compounds be incorporated in the oil in greater amounts, i. e. above 10%, to provide "concentrates" for marketing. These concentrated compositions have the advantage of affording a readily soluble form of the additive compound for dilution with additional quantities of oil prior to actual use.

The oils in which our new addition agents are used, or the oil "concentrates," may also contain other additives, designed to improve the character of the oil in other respects, such as detergency, V. I. antioxidant quality, etc.

Having now fully described our invention what we wish to claim as new and patentable is:

1. A mineral lubricating oil containing a minor proportion, sufficient to depress the pour point thereof, of a polymeric n-tetradecyl metaphosphimate product obtained by (1) reacting a phosphonitrilic halide with n-tetradecanol at a temperature not in excess of about 150° C. to form n-tetradecyl metaphosphimate and (2) subjecting the metaphosphimate to polymerization by 50 the method selected from (a) further heating the

Table I

| Ex. No. | Reaction Product                                            | ASTM Pour Point |      |      |
|---------|-------------------------------------------------------------|-----------------|------|------|
|         |                                                             | 1%              | 1/2% | 1/4% |
| I       | $(\text{PNCl}_2)_3 + 2(\text{Lorol-B})\text{ONa}$           | +15             |      |      |
| II      | $(\text{PNCl}_2)_3 + 2\text{C}_{10}\text{H}_{21}\text{ONa}$ | +20             | +25  |      |
| III     | $(\text{PNCl}_2)_3 + 2\text{C}_{12}\text{H}_{25}\text{ONa}$ |                 | +20  | +20  |
| IV      | $(\text{PNCl}_2)_3 + 2\text{C}_{14}\text{H}_{29}\text{ONa}$ | +25             |      |      |
| V       | $(\text{PNCl}_2)_3 + 2\text{C}_{16}\text{H}_{33}\text{ONa}$ | +25             | +15  |      |
| VI      | $(\text{PNCl}_2)_3 + 2\text{C}_{18}\text{H}_{37}\text{ONa}$ | +30             | +20  |      |

Table II

| Ex. No. | Reaction Product Polymerized with $\text{AlCl}_3$           | ASTM Pour Point |      |      |      |
|---------|-------------------------------------------------------------|-----------------|------|------|------|
|         |                                                             | 1%              | 1/2% | 1/4% | 1/6% |
| I-A     | $(\text{PNCl}_2)_3 + 2(\text{Lorol-B})\text{ONa}$           | -30             | -30  | -30  | -10  |
| II-A    | $(\text{PNCl}_2)_3 + 2\text{C}_{10}\text{H}_{21}\text{ONa}$ | +15             | +15  |      |      |
| III-A   | $(\text{PNCl}_2)_3 + 2\text{C}_{12}\text{H}_{25}\text{ONa}$ | +15             | +20  |      |      |
| IV-A    | $(\text{PNCl}_2)_3 + 2\text{C}_{14}\text{H}_{29}\text{ONa}$ | -25             | -20  | -15  | -5   |
| V-A     | $(\text{PNCl}_2)_3 + 2\text{C}_{16}\text{H}_{33}\text{ONa}$ | +20             | +15  |      |      |
| VI-A    | $(\text{PNCl}_2)_3 + 2\text{C}_{18}\text{H}_{37}\text{ONa}$ | +15             | +15  |      |      |

metaphosphimate product at a temperature not in excess of 150° C. in the presence of a polymerization catalyst, and (b) heating the metaphosphimate product at a temperature ranging from about 200° C. to about 400° C.

2. A mineral lubricating oil containing a minor proportion, sufficient to depress the pour point thereof, of a polymeric n-tetradecyl metaphosphimate product obtained by reacting phosphonitrilic chloride with n-tetradecanol at a temperature not in excess of about 150° C. to form an n-tetradecyl metaphosphimate and then subjecting the metaphosphimate to polymerization by the method selected from (a) further heating the metaphosphimate at a temperature not in excess of 150° C. in the presence of an aluminum chloride catalyst, and (b) heating the metaphosphimate at a temperature ranging from about 200° C. to about 400° C.

3. A mineral lubricating oil containing a minor proportion, sufficient to depress the pour point thereof, of a polymeric alkyl metaphosphimate product produced by (1) reacting a phosphonitrilic halide with a mixture of primary, normal, saturated alcohols, said mixture consisting of alcohols containing from 10 to 18 carbon atoms in the following approximate proportions

Per cent  
 $C_{10}=2.5$   
 $C_{12}=55.0$   
 $C_{14}=20.5$   
 $C_{16}=9.0$   
 and  $C_{18}=13.0$

to form an alkyl metaphosphimate and (2) subjecting the metaphosphimate to polymerization by the method selected from (a) further heating the metaphosphimate product at a temperature

not in excess of 150° C. in the presence of a polymerization catalyst, and (b) heating the metaphosphimate product at a temperature ranging from about 200° C. to about 400° C.

4. A mineral lubricating oil containing a minor proportion, sufficient to depress the pour point thereof, of a polymeric alkyl metaphosphimate product produced by (1) reacting a phosphonitrilic halide with a mixture of primary, normal, saturated alcohols, said mixture consisting of alcohols containing from 10 to 18 carbon atoms in the following approximate proportions

Per cent  
 $C_{10}=2.5$   
 $C_{12}=55.0$   
 $C_{14}=20.5$   
 $C_{16}=9.0$   
 and  $C_{18}=13.0$

20 to form an alkyl metaphosphimate and (2) subjecting the metaphosphimate to polymerization by the method selected from (a) further heating the metaphosphimate product at a temperature not in excess of 150° C. in the presence of an aluminum chloride catalyst, and (b) heating the metaphosphimate product at a temperature ranging from about 200° C. to about 400° C.

FERDINAND P. OTTO.  
 ROBERT W. BARRETT.

#### REFERENCES CITED

The following references are of record in the file of this patent:

#### UNITED STATES PATENTS

| Number    | Name   | Date         |
|-----------|--------|--------------|
| 2,109,491 | Lipkin | Mar. 1, 1938 |